

# UNITED STATES PATENT OFFICE.

MARTIN BOEHLER, OF FRANKFORT-ON-THE-MAIN, GERMANY, ASSIGNOR TO  
LEOPOLD CASSELLA & CO., OF SAME PLACE.

## PROCESS OF DYEING DARK BLUE.

SPECIFICATION forming part of Letters Patent No. 625,717, dated May 23, 1899.

Application filed December 10, 1898. Serial No. 698,882. (No specimens.)

*To all whom it may concern:*

Be it known that I, MARTIN BOEHLER, a citizen of Prussia, and a resident of Frankfort-on-the-Main, Hesse-Nassau, Germany, have invented certain new and useful Improvements in the Production of Blue Shades on Cotton, of which the following is a specification.

I have found that dyeings produced with the dyestuffs commercially named "immedial blacks," which are described in the United States Letters Patent No. 610,541, dated September 13, 1898, and derived from oxydinitrodiphenylamin, sulfid of sodium, and sulfur, if treated with hydrogen dioxid will change their shades to a dark blue. The thus obtained dyeings are distinguished by their great fastness to washing, acids, light, chlorin, &c.

Example: Twenty kilos cotton are dyed at a temperature of 80° centigrade in a bath of four hundred liters water containing one kilo immedial black V. extra, eight-tenths kilo sodium sulfid, and twelve kilos common salt. The cotton is allowed to remain in the bath during about one hour, then lifted and rinsed, then

entered into a second bath, to which some ammonia—two liters of a solution containing ten per cent. of hydrogen dioxid—has been added. The reaction is terminated after treating the cotton for about one-half hour 30 in this bath at a temperature of about 80° centigrade.

Having thus described my invention and in what manner the same can be performed, what I claim as new, and desire to secure by 35 Letters Patent, is—

The process of producing dark-blue shades on the cotton fiber by treating with hydrogen dioxid the dyeings done with the dyestuffs derived by heating oxydinitrodiphenylamin 40 with sulfid of sodium and sulfur, substantially as described.

Signed at Frankfort-on-the-Main, in the Province of Hesse-Nassau and Empire of Germany, this 25th day of October, A. D. 1898. 45

MARTIN BOEHLER.

Witnesses:

JEAN GRUND,  
FRANK H. MASON.